

# United States Patent [19]

Ludwigson

[11] 3,926,692  
[45] Dec. 16, 1975

[54] **DRAWABILITY OF DEOXIDIZED STEELS  
BY THE ADDITION OF PHOSPHORUS AND  
SILICON**

[75] Inventor: **David C. Ludwigson, Hempfield  
Township, Westmoreland County,  
Pa.**

[73] Assignee: **United States Steel Corporation,  
Pittsburgh, Pa.**

[22] Filed: **Sept. 30, 1974**

[21] Appl. No.: **510,844**

[52] **U.S. Cl. .... 148/36; 75/123 R**

[51] **Int. Cl. .... C22C 38/00**

[58] **Field of Search .... 75/123 R; 148/2, 3, 12,  
148/36**

[56] **References Cited**

UNITED STATES PATENTS

3,215,567 11/1965 Yoshida .... 75/123 R X

|           |         |                              |
|-----------|---------|------------------------------|
| 3,522,110 | 7/1970  | Shimizu et al. .... 148/12 C |
| 3,668,016 | 6/1972  | Shimizu et al. .... 148/12 C |
| 3,709,744 | 1/1973  | Goodman et al. .... 148/36   |
| 3,806,373 | 4/1974  | Shimizu et al. .... 148/12 C |
| 3,843,415 | 10/1974 | Leslie..... 148/2            |

FOREIGN PATENTS OR APPLICATIONS

725,104 1/1966 Canada ..... 148/36

*Primary Examiner*—C. Lovell  
*Attorney, Agent, or Firm*—Arthur J. Greif

[57] **ABSTRACT**

The high drawability of deoxidized steels with Mn contents below about 0.22 percent is enhanced by the addition of from about 0.015 to 0.05 percent P. The beneficial effect of such phosphorus additions on drawability is further enhanced by employing from about 0.02 to 0.06 percent Si.

**2 Claims, 2 Drawing Figures**



FIG. 1. MANANESE CONTENT WT %



FIG. 2. WT % SILICON

## DRAWABILITY OF DEOXIDIZED STEELS BY THE ADDITION OF PHOSPHORUS AND SILICON

This invention relates to an economical sheet steel product with exceptionally high deep drawability, as evidenced by  $r$  value, and is more particularly related to a specific range of steel compositions which will provide such deep drawability.

It is generally recognized that the performance of a sheet steel during forming operations known as deep drawing is closely associated with the ratio,  $r$ , of true width strain to true thickness strain when the steel is strained in tension in the length direction. Therefore, the suitability of a steel for deep drawing may be assessed by measuring  $r$  in the laboratory and the greater difficulty of full scale drawing trials can often be averted. It is normal to measure  $r$  in the plane of the sheet in three directions, parallel to the rolling direction ( $r_0$ ), diagonal to the rolling direction ( $r_{45}$ ), and perpendicular to the rolling direction ( $r_{90}$ ). From these three components, two summary characteristics are usually derived:

$$\bar{r} = (r_0 + 2r_{45} + r_{90})/4 \quad (1)$$

$$\Delta r = (r_0 - 2r_{45} + r_{90})/2 \quad (2)$$

High values of  $\bar{r}$  are associated with a high capability to undergo deep drawing with fracture; and values of  $\Delta r$  near zero are associated with a low tendency toward a detrimental directional nonuniformity in deep drawn items known as earing.

Isotropic steels have been produced with  $\bar{r}$  and  $\Delta r$  values near 1.0 and 0.0, respectively. Such steels have limited deep drawability but excellent resistance to earing. Cold-rolled rimmed sheet steels generally exhibit  $\bar{r}$  and  $\Delta r$  of about 1.2 and +0.4, respectively. Such steels can be subjected to mild deep drawing operations, but develop detrimental earing. Drawing-quality special-killed (DQSK) steels are often characterized by  $\bar{r}$  and  $\Delta r$  values near 1.5 and +0.5, respectively. Although these steels can withstand severe draws, they too tend to suffer from earing; and they are more costly to produce than rimmed steels. Recently sheet steels containing columbium or titanium to combine with interstitial elements have appeared. These steels have  $\bar{r}$  values of 2.0 or more and thus can withstand very severe deep drawing. Earing tendency may be small in some instances, as indicated by  $\Delta r$  values near -0.1, or high in other instances, as indicated by  $\Delta r$  values near +0.5. However, because of their columbium or titanium contents, these steels are very costly to produce. A significantly more economical method for improving deep drawability is through the addition of phosphorus to unkillled steels. Thus, U.S. Pat. Nos. 3,215,567 and 3,244,565 show that the addition of greater than about 0.03 percent phosphorus to an unkillled steel, followed by a decarburization of the sheet product, can significantly improve deep drawability. However, the  $r$  values of these steels only approach those of the above noted DQSK steels.

It is therefore a principal object of this invention to provide a phosphorus containing steel composition which can yield sheet products with  $\bar{r}$  values of the order of 2.0 and greater.

It is a further object of this invention to provide a phosphorus containing steel composition which can provide superior drawability without the need for decarburization, i.e., in which the carbon content of the final product is greater than 0.010 percent.

These and other objects will be more readily understood from a reading of the following description when read in conjunction with the appended claims and drawings, in which:

5 FIG. 1 shows the interacting effects of Mn and P on  $r$  value, and

FIG. 2 shows the beneficial effect, on  $\bar{r}$  value, of Si additions to a phosphorus containing steel.

The anisotropy that results in favorable  $\bar{r}$  and  $\Delta r$  values is developed through metallurgical reactions in the steel that favor certain orientations of individual grains in the steel with respect to the steel surface and rolling direction. In particular, when a high fraction of grains are oriented with their  $<111>$  axes perpendicular to the face of the sheet, high  $\bar{r}$  values are observed. To determine the effect on such orientations, of those residual elements which are normally found in sheet steels, a series of heats were prepared with planned variations of the following elements; manganese, phosphorus, sulfur, silicon, copper, nickel, oxygen and nitrogen. Each heat was finish hot-rolled to a nominal thickness of 0.09 inch, at a temperature of about 1650°F and the resultant band slow cooled from 1150°F to simulate the thermal history of commercial coiled product. After descaling, each band was cold reduced to a nominal thickness of 0.030 inch, i.e., to an aim cold reduction of about 67 percent. The resultant cold-reduced strips were recrystallization-annealed in conventional manner and subsequently evaluated for

30 both  $\bar{r}$  and  $\Delta r$  values. From the data on the experimental steel compositions, and with the use of regression analysis; the relationship of  $\bar{r}$  and  $\Delta r$  as a function of the levels of the above noted alloy elements was derived. It was found that within the ranges tested, that the elements sulfur copper, nickel, oxygen and nitrogen were all detrimental to the achievement of high  $\bar{r}$  values. Stated another way, increasing the level of any of the foregoing five elements had an inverse effect on  $\bar{r}$  value. In view thereof, it is desirable that the aforementioned steelmaking impurities be maintained at levels less than the following specified maximums: 0.04 percent S, preferably 0.03 percent max.; 0.05 percent Cu; 0.12 percent Ni; 0.015 percent N, preferably 0.01 max.; and 0.02 percent oxygen, preferably 0.015 percent max. However, in distinction to the teachings of the aforementioned U.S. Pat. Nos. (3,215,567 and 3,244,565) it was found that phosphorus can enhance the drawability of killed (deoxidized) steels, as well. However, with killed steels P will only be beneficial if

50 the Mn level is maintained below about 0.22 wt. percent. The rather surprising interaction between Mn and P in a deoxidized steel will be more readily understood by reference to FIG. 1. It may be seen, in accord with the teaching of U.S. Pat. No. 3,215,567 (eg. compare thereto steels 17 vs 18) that for a "killed steel" in which the level of Mn is, for example, 0.35 percent, that an increase in the level of phosphorus will have a significant, detrimental effect on drawability. With compositions containing from 0.22 to 0.28, the level of P has

55 only a slight or negligible effect on  $\bar{r}$  value. More importantly, however, with Mn levels of about 0.22 percent or less, the  $\bar{r}$  value materially increases with increasing phosphorus contents; this beneficial effect of phosphorus becoming even more pronounced with progressively decreasing manganese contents.

In view of this "flip-flop" effect of P in "killed steels" depending on Mn content, it may therefore be surmised why the above noted prior art teachings as to the bene-

ficial effects of P are limited to "unkilled" steels. The reduction of Mn to levels below about 0.2 percent is not only expensive, but may be detrimental in that there generally would be an insufficient amount to bind up the S present in steel; thereby rendering the steel

measured and calculated strain-ratio values. Example 1, provided for comparison, is a control sample wherein p is outside the scope of this invention. Examples 2 and 3 are compositions within the scope of this invention.

Table I

| No. | C     | Mn    | P     | S     | Si    | Cu     | Ni    | Mo     | N     | Al(total) | O(ppm) |
|-----|-------|-------|-------|-------|-------|--------|-------|--------|-------|-----------|--------|
| 1   | 0.012 | 0.08  | 0.006 | 0.006 | 0.020 | 0.040  | 0.114 | 0.004  | 0.003 | 0.004     | 151    |
| 2   | 0.011 | 0.075 | 0.020 | 0.006 | 0.042 | <0.005 | 0.022 | <0.005 | 0.002 | 0.002     | 175    |
| 3   | 0.011 | 0.085 | 0.021 | 0.005 | 0.056 | 0.040  | 0.025 | <0.005 | 0.003 | 0.005     | 144    |

subject to edgecracking (hot-shortness). Thus, the art has only employed low Mn levels when it was absolutely required, i.e., for improving the sag-resistance of enameling steels. Equally important, until recently, such low Mn steels were not capable of being recrystallized by a subcritical anneal. Thus, it was necessary that such low Mn steels be recrystallized by normalizing; a treatment which would destroy the attainment of high  $\bar{r}$  values. It is, of course, now known (e.g. U.S. Pat. Nos. 3,668,016 and 3,709,744) that such low Mn steels can be subcritically annealed if they are deoxidized to a requisite extent and that such lower levels of Mn are in fact beneficial for the production of high  $\bar{r}$  values. Therefore, the investigations of U.S. Pat. Nos. 3,215,567 and 3,244,565 were probably limited to the effect of P in steels with Mn levels above about 0.25 percent. However, in (deoxidized) steels with such higher Mn levels, it may be seen that increasing the P content will actually decrease the  $\bar{r}$  value attained, i.e., FIG. 1, and U.S. Pat. No. 3,215,567, noted above.

Additionally, it was found that higher levels of Si also enhanced drawability; with the beneficial effect increasing progressively as the P content was increased. This latter relationship is shown in FIG. 2. Referring to that figure, it may be seen that a P level of 0.01 percent, an increase in Si content provides some increase in  $\bar{r}$  value. However, at a P level of 0.02 percent or greater, 40 an increase in Si provides a rather dramatic increase in  $\bar{r}$  value.

Three steel heats of varying compositions were processed to sheet, in the manner outlined above. The specific compositions of the resultant sheet products are shown in Table I, while Table II presents both the

Table II

| No. | $r_0$ | Strain-Ratio Values |          |           | $\bar{r}$ | $\Delta r$ |
|-----|-------|---------------------|----------|-----------|-----------|------------|
|     |       | $r_{45}$            | $r_{90}$ | $\bar{r}$ |           |            |
| 1   | 1.581 | 1.795               | 2.291    | 1.866     | 0.141     |            |
| 2   | 1.891 | 2.227               | 2.573    | 2.230     | +0.005    |            |
| 3   | 1.760 | 2.306               | 2.844    | 2.304     | -0.004    |            |

Aside from their somewhat lower Ni contents, it may be seen that examples 2 and 3 are essentially the same composition as the control, except for their higher P and Si contents. The decidedly higher  $\bar{r}$  values of the latter two examples, is clearly evident. It is also noteworthy that such high  $\bar{r}$  values have been achieved without any sacrifice in directional uniformity, i.e.,  $\Delta r$ 's very near to zero.

I claim:

1. A deep drawable killed-steel sheet product exhibiting an  $\bar{r}$  value of at least about 2.0, the composition of which consists essentially of, in weight percent,

|        |             |
|--------|-------------|
| C      | 0.010 - 0.1 |
| Mn     | 0.22 max.   |
| P      | 0.03 - 0.05 |
| Si     | 0.02 - 0.06 |
| oxygen | 0.02 max.   |

balance Fe and incidental steelmaking impurities, said product having been produced from a steel melt which was killed in order to reduce the oxygen content thereof to said maximum percentage.

2. The sheet product of claim 1 wherein oxygen is 45 below about 0.015 percent.

\* \* \* \* \*